

J. C. DAVIS.

CASTING APPARATUS AND PROCESS.

APPLICATION FILED OCT. 7, 1909. RENEWED OCT. 18, 1915.

1,192,044.

Patented July 25, 1916.



WITNESSES

Geo. C. Garrison  
Maurice Goldberger.

INVENTOR

James Barry Davis  
By Attorneys  
Cynamon, Tredt & Carpenter

# UNITED STATES PATENT OFFICE.

JAMES CAREY DAVIS, OF HINSDALE, ILLINOIS.

## CASTING APPARATUS AND PROCESS.

1,192,044.

Specification of Letters Patent. Patented July 25, 1916.

Application filed October 7, 1909, Serial No. 521,622. Renewed October 18, 1915. Serial No. 56,595.

To all whom it may concern:

Be it known that I, JAMES CAREY DAVIS, a citizen of the United States, and a resident of Hinsdale, in the county of DuPage 5 and State of Illinois, have invented certain new and useful Improvements in Casting Apparatus and Processes, of which the following is a specification.

My present invention relates to the art 10 of casting metal and to means for introducing a hardening or other modifying element into the molten metal before it flows into the mold, and has special reference to the provision of improved means whereby the 15 admixture and distribution of the modifying element may be regulated and determined with nicety, to the end that not only a homogeneity of metal throughout the casting, or certain parts thereof, may be secured but also that the repeated reproduction 20 of a run of castings of like composition may be attained.

The principal objects of my invention are the provision of improved apparatus for 25 the present purposes, which will most uniformly and thoroughly mix the molten metal and the modifying element, and do so more fully and completely than had heretofore been done in any manner known to 30 me, and do so more effectively than it has been possible to do it by pouring of the modifying element into or adjacent to the stream of molten metal as it enters the gate of the mold; and to provide means whereby 35 the size and velocity of the stream of molten metal may be made uniform and constant to the end that the proportion of the modifying element introduced thereto may be more closely controlled, and consequently 40 castings of a more closely predetermined composition produced, together with further objects to be below disclosed.

My invention further contemplates the utilization of an improved process of making castings, which may if desired be of differing degrees of hardness in different portions, such as those made of steel which is hard and resistant and consequently of good wearing qualities at the exterior and 50 comparatively softer toward the center, and therefore more tough and less likely to fracture, such process being useful for the production of cast steel wheels and other structures.

55 In the production of castings containing a modifying element, by other apparatus and processes known to me, I have experi-

enced great difficulty in insuring a constant proportion between the principal metallic element forming the body of the casting, 60 and the modifying element introduced thereto, owing to the tendency of the molten metal as it comes from the furnace, cupola or ladle to flow in a stream of irregular contour, as it tends to spurt or spread out in 65 the form of a hollow cone or umbrella-like spray instead of descending in a solid column, which not only renders it difficult to properly apportion the modifying element to the stream but often renders it impossible to thoroughly incorporate the modifying element with all parts of the flowing metal.

In the accomplishment of the foregoing objects and in the avoidance of the disadvantages above mentioned as well as to attain such other advantages as may herein-after appear, I have provided a construction one form of which I have illustrated in the accompanying drawings, wherein— 80

Figure 1 is an elevation partly in section of a rotatable mold wherein a casting may be made in accordance with my invention; Fig. 2 is a plan view of certain parts shown in Fig. 1; and Fig. 3 is a view of a detail 85 of construction.

Referring first to Fig. 1 it will be noted that in carrying out my invention I mount in a convenient place, as in a pit 10, the desired number of molds 11 each of which is 90 mounted upon a rotatable table 12 supported by a vertical shaft 13 carrying a gear 14 driven by a pinion 15. Upon the upper flask member 16 I arrange a pouring gate 17 provided with a refractory lining 18. 95

For the purpose of providing means whereby the molten metal from the ladle 23 may be maintained at a height substantially uniform and will thereby be caused to descend in a solid column of uniform 100 diameter, contour and velocity, I provide a choke device comprising a hopper or funnel 19, preferably conically shaped, the open bottom of which is partially closed by a nozzle 20 which is formed of refractory material and may be renewed from time to time as required in service. To the end that the choke device may be centered over the pouring gate 17, and where circumstances render it desirable moved from one flask to another, it is mounted upon a truck 21 which comprises a supporting bed 22 carried upon axles 24 the wheels of which 25 are revolute thereupon and arranged to ride upon 105 110

rails 26 the outer ends of which are mounted upon trucks 27 and 28 which in turn ride upon the rails 29 and 30 oppositely disposed about the molds 11.

5 For the purpose of introducing and incorporating most perfectly and commingling and distributing most thoroughly the modifying element into the stream of flowing metal 31, which, as will be seen, on reference to Fig. 1 takes the form substantially of a column with parallel sides, I make use 10 of an apparatus which here comprises a vertical casing 32 for containing the modifying elements, such as manganese, chromium, vanadium, etc., a lateral extension thereof 15 33, a nozzle 34 the ejector of which, 35 (Fig. 3) is depressed somewhat from the horizontal, and a pipe 36 connected to a source of air or other fluid pressure supply, and inserted into the apparatus below the casing 20 32 to the end that the modifying element may be drawn therefrom by fluid pressure and forced into the flowing stream of metal. In practice, I have found that the best 25 results are attained by the use of pressures between approximately 50 and 125 lbs. per square inch which will cause the modifying element to penetrate the stream of molten metal, and that by flattening the ejector 35 30 so that the spray of modifying material may be spread out to approximately the diameter of the stream, and depressing the end of the ejector so that the modifying material will strike the flowing stream in the direction in 35 which it flows, it will enter and be more thoroughly commingled and homogeneously incorporated with the molten metal, and will not have the tendency to become segregated in masses therein nor to be unevenly disposed 40 therein, nor to remain on the surface of the stream and subject to the action of the air.

While I have illustrated my invention in connection with a rotating mold 4, available 45 for the manufacture of wheels, and believe that it is particularly useful for the production of such articles and others wherein it is desirable to have a greater portion of the modifying element toward the periphery, my invention is useful for the manufacture 50 of castings in stationary molds, or intermittently rotated molds, wherein are made castings of either a homogeneous composition throughout or those formed of a number 55 of strata of material.

The use of pressures of the strength above indicated is in my experience preferable to either lower or higher pressures as it insures penetration of the surface of the stream on 60 one hand without the disadvantages which are obviously incident to the use of jets of greater force.

From the foregoing description it will be manifest that one of the problems which has been solved by my present invention is the

problem of accurately and uniformly proportioning the quantities of the modifying element and molten metal as they enter the mold. In order to do this, obviously it is not only desirable to have the modifying element delivered in uniform and unvarying quantity, but it is also desirable to have the molten metal delivered in uniform and unvarying quantity. If the metal be taken directly from a pouring ladle of the ordinary type its velocity will vary as the height of the metal in the ladle varies. From this it follows that if the rate of flow of the modifying element be uniform, the proportion of the modifying element and metal delivered to the mold will vary, because the rate of flow of the metal is not uniform. In overcoming this I have provided a choke device whereby I am enabled to maintain the height of the metal in that device substantially uniform. As a result, the discharge of metal into the mold is uniform. Furthermore, as the head of metal in the choke device is relatively small, the issuing stream is in the form of a substantially solid column. Furthermore, by employing the injecting device referred to, the modifying element is immediately embedded in and firmly held by the flowing metal, and is therefore uniformly carried into the mold.

It is believed that the operation of my invention will be understood without further detailed description, and that other advantages of my invention and other specific means of choking the stream of molten metal and of directing the spray of modifying element will occur to those who are skilled in the art to which my invention pertains.

Having thus described my invention and illustrated its use what I claim as new and desire to secure by Letters Patent is the following:

1. The combination with a rotatable mold, a ladle, and means for rotating the mold, of a choke device whereby the flow of metal from the ladle to the mold may be governed, and a device for introducing a modifying element into the stream of metal as it comes from the choke device.

2. The combination with a mold and a ladle, of a choke device whereby the flow of metal from the ladle to the mold may be governed, said choke device being supported by a truck movable on rails which in turn are movably supported by other rails.

3. The combination with a mold and a ladle, of a portable choke device supported on a truck and traveling on wheels, and a device for introducing a modifying element into the flowing metal as it runs toward the mold, such introducing device being situated for use between said choke device and the gate of the mold, substantially as described.

4. The combination of a choke device for

governing the flow of metal to a mold, and a device for introducing a modifying element into the stream of metal as it comes from the choke device.

5. The combination of a choke device for governing the flow of metal to a mold and a ladle, the choke device having a discharge orifice smaller than the discharge orifice of the ladle.

10. The combination with a ladle, a mold, and a device for introducing a modifying element into the metal as it flows toward the mold, of a choke device between the ladle and the introducing device, said choke device having a discharge orifice smaller than the discharge orifice of the ladle.

15. In a casting apparatus the combination with a choke device having an aperture to permit the efflux of molten metal, of a device for introducing a modifying element into the flowing stream of metal in a spray of substantially the same width as the stream of metal from the choke device.

20. The combination with a mold and ladle, of a device for introducing a modifying element into the flowing stream of metal, comprising a source of fluid pressure supply, a container for the modifying element and a nozzle having a relatively long orifice of a 30 restricted cross section, whereby the modifying element may be delivered in the form of a spray.

25. The combination with a mold and ladle, of a device for introducing a modifying element into the flowing stream of metal, comprising a connection to a source of fluid pressure supply, a container for the modifying element and a lateral connection from the container terminating in an ejector 35 nozzle, the said pressure connection being arranged to draw material from the container and eject it through the nozzle.

30. The process of introducing a modifying element into a cast body during the pouring into the mold which consists in causing the molten metal to enter the mold in the form of a substantially solid column and forcing the modifying element into the descending column between the ladle and 45 the mold.

35. The process of introducing a modifying element into a cast body during the pouring into the mold, which consists in choking the flowing metal into a stream of 50 substantially continuous size and uniform velocity and forcing the modifying element into the stream between the choke device and the mold.

40. The process of introducing a modifying element into a cast body during the pouring into the mold, which consists in choking the flowing metal into a stream of 55

substantially continuous size and uniform velocity and forcing the modifying element into the stream in the direction of travel of such metal between the choke device and the mold.

60. The process of introducing a modifying element into a cast body during the pouring into the mold which consists in maintaining the molten metal at a height substantially uniform and causing the molten metal to enter the mold in the form of a substantially solid column and forcing the modifying element into the descending column between the ladle and the mold.

65. The process of introducing a modifying element into a cast body during the pouring into the mold which consists in maintaining the molten metal at a height substantially uniform and causing the molten metal to enter the mold in the form of a substantially solid column and forcing the modifying element into the descending column between the ladle and the mold, and rotating the mold.

70. The process of introducing a modifying element into a cast body during the pouring into the mold, which consists in maintaining the molten metal at a height substantially uniform and choking the flowing metal into a stream of substantially continuous size and uniform velocity and forcing the modifying element into the stream between the choke device and the mold; and rotating the mold.

75. The process of introducing a modifying element into a cast body during the pouring into the mold, which consists in maintaining the molten metal at a height substantially uniform and choking the flowing metal into a stream of substantially continuous size and uniform velocity and forcing the modifying element into the stream in the direction of travel of such metal between the choke device and the mold, and rotating the mold.

80. The process of introducing a modifying element into a cast body during the pouring into the mold which consists in maintaining the molten metal at a height substantially uniform and causing the molten metal to enter the mold in the form of a substantially solid column and forcing the modifying element into the column between the ladle and the mold, and rotating the mold.

85. In testimony whereof I have hereunto signed my name in the presence of the two subscribed witnesses.

JAMES CAREY DAVIS.

Witnesses:

PAUL CARPENTER,  
DONALD C. WILLIAMS.